

April 2, 1974

HIROYUKI YAMAGUCHI ET AL  
ANTISTATIC ACRYLIC SYNTHETIC FIBERS AND A  
PROCESS FOR THE MANUFACTURE THEREOF  
Original Filed Dec. 22, 1969

3,801,553



1

3,801,553

ANTISTATIC ACRYLIC SYNTHETIC FIBERS AND  
A PROCESS FOR THE MANUFACTURE THEREOF  
Hiroyuki Yamaguchi, Kyoto, and Shigeyuki Komure,  
Ibaraki, Japan, assignors to Asahi Kasei Kogyo Kabu-  
shiki Kaisha, Osaka, Japan  
Continuation of abandoned application Ser. No. 887,215,  
Dec. 22, 1969. This application Oct. 5, 1971, Ser. No.  
186,810

Claims priority, application Japan, Dec. 20, 1968,  
43/93,139

Int. Cl. C08f 29/52, 45/00

U.S. CL. 260—79.3 MU

13 Claims

## ABSTRACT OF THE DISCLOSURE

An acrylic synthetic fiber comprising at least 70% by weight acrylonitrile and from 2 to 10% by weight of at least one polyalkylene ether derivative represented by the formula:



wherein R is a hydrophobic organic radical of from 6 to 40 carbon atoms derived from a compound having a —OH or a —COOH group by removing said —OH or said —COOH group; R' is hydrogen or methyl; X is O or COO; n is an integer larger than 2 and m is an integer of from 1 to 6. Also disclosed is a process for making such acrylic synthetic fibers comprising wet-spinning a polymer comprising at least 70% acrylonitrile into filaments, contacting the resulting filaments with the above-identified polyalkylene ether derivative with an amount of the derivative, based on the dry weight of the fibers, larger than that amount of the derivative, based on the dry weight of the fibers, which remains in the fibers after the fibers have been treated in boiling water for at least one hour.

## CROSS-REFERENCE TO RELATED APPLICATION

The present application is a continuation of U.S. application Ser. No. 887,215, filed Dec. 22, 1969, now abandoned, claiming priority from Dec. 20, 1968 based on Japanese patent application Ser. No. 93,139/1968.

This invention relates to an improved acrylic synthetic fiber having not only superior fiber characteristics, but also a highly favorable antistatic performance, and a process for the manufacture of such improved acrylic synthetic fibers.

While acrylic synthetic fibers possess favorable physical characteristics for use as textile materials and superior dyeing behavior, they show a strong tendency toward static characteristics.

Substantial troubles are therefore encountered during manufacture and use of acrylic synthetic fibers on account of the static charges accumulated therein by frictional contact between the fibers.

Various prior methods are known for the prevention of the accumulation of static charges in the acrylic man-made fibers. As an example, an antistatic agent selected

2

from the group of known surfactants is used for the treatment of such fibers for attaining the desired effect, but it has been experienced that the thus applied antistatic agent is frequently removed off even upon a single washing. Therefore, the antistatic effect thus attained is not permanent. For obviating such a conventional drawback, it has also been proposed to use a certain kind of hydrophilic high molecular weight compound as the antistatic agent; however the results leave much to be desired with respect to the wash fastness of the fibers.

It is therefore the main object of the invention to provide a highly durable antistatic acrylic fiber which possesses superior physical characteristics per se.

It is now been found that if an acrylic fiber comprising an acrylic polymer contains in a suitable way at least 2 wt. percent of at least one member selected from the group consisting of polyalkylene ether derivatives represented by the general formula:



where

R stands for a hydrophobic organic radical having 6-40 carbon atoms; R' for a hydrogen or methyl group; and X for an oxygen atom or an ester bond, n being an integer larger than 2 and m also being an integer of 1-6,

the fiber has a superior antistatic performance, indeed, without any substantial loss of the originally owned fiber properties adapted for use as a textile fabric material.

The term "acrylic polymer" as used throughout the present specification and appended claims stands for an acrylonitrile polymer per se, or a copolymer comprising at least 70 wt. percent of acrylonitrile and a monomer carrying another unsaturated radical or radicals.

Representative comonomers usable for the above purpose may be, among others, as follows: methacrylic acid; methyl acrylate; butyl acrylate; methyl methacrylate; ethyl methacrylate; butyl vinyl ether; acrylic acid ester; methacrylic acid ether; vinyl ether; vinyl acetate ester; styrene sulfonic acid; sodium styrene sulfonate; sodium allylsulfonate; sodium methallyl sulfonate. These examples are not intended to limit the present invention and other comonomers which are commonly used in the textile industry are also usable in the practice of the invention.

As was referred to hereinabove, the hydrophobic organic group of the polyalkylene ether derivatives should have 6-40 carbon atoms. With such polyalkylene ether derivatives having an organic radical with less than 6 carbon atoms, the desired effect would not be sufficient for the purpose aimed at, and indeed, on account of insufficiency of the hydrophobic performance of the organic radical.

When the number of carbon atoms exceeds 40, the molecule will become too large which results in unfavorable results. Such hydrophobic organic radicals (expressed by R) may be derived from compounds where the radicals are associated with the X radical and the hydrogen atom, and thus each of the compounds carry an —OH or an —COOH group; and the compounds may preferably be compounds such as octyl alcohol, dodecyl alcohol,

hexadecyl alcohol, octadecyl alcohol, octadecenyl alcohol, octylphenol, dodecylphenol, stearic acid monoglyceride, ricinoleic acid triglyceride, sorbitan oleate, sorbitan distearate, octanoic acid, dodecanoic acid,  $\omega$ -hydroxy decanoic acid, sebacic acid,  $\alpha$ - or  $\omega$ -dihydroxy octane, methylene bis-phenol and the like. This kind of compound may be an isolated one, or in the form of a natural mixture such as castor oil, tallow, fatty acid or the like.

The polyalkylene ether derivative usable in the present invention comprises a hydrophobic organic radical added with polyoxyethylene-, polyoxypropylene- or both. The degree of polymerization of the alkylene ether should preferably be 2-200, preferably less than 50. The polyalkylene ether derivative under consideration can be prepared easily by subjecting the hydrophobic compound carrying an OH- or COOH radical, in the form of one side starting material, with ethylene oxide or propylene oxide as the other side material.

The acrylic synthetic fiber according to this invention should preferably contain at least 2 wt. percent of the derivative relative to the polymer constituting the fiber. With a content considerably less than 2 wt. percent, the desired effect would be insufficient. The possible upper limits of the content depends naturally upon the kind and nature of the fiber, the method of preparation and the kind and nature of the polyalkylene ether derivative under consideration, the degree of the desired effect, and the like, and will amount generally to about 10%.

There are various ways for the addition of the polyalkylene ether derivative to the acrylic fiber. As a measure, the derivative may be added to the spinning solution and the mixture is then spun into filamentary fibers according to a wet or dry spinning process, as the case may be.

The most preferable way for the addition of the polyalkylene ether derivative to the acrylic fiber is to immerse the latter in an aqueous solution of said derivative. For this purpose, the acrylic fiber in a wet gel state is immersed, preferably at 20-30° C., in an aqueous bath containing the polyalkylene oxide derivative and then mangled or centrifuged at room temperature. When the derivative under consideration is liquid per se, the acrylic fiber in its wet gel state and the antistatic agent in the form of said kind of derivative may advantageously be brought into direct contact with each other. If the agent is insoluble in water, a solvent or dispersing agent may be adopted.

In any case, the contacting period between the fiber and the antistatic agent per se or in solution may extend from a shortest time such as one second to a considerable time length such as several tens minutes. The bath may naturally contain one or more of various conventional fiber-improving additives. Anyhow, by adopting any one of the above-mentioned treating ways, the antistatic agent may be included within the fibers.

It will be seen from the foregoing that according to this invention a considerable amount of polyalkylene ether derivative is given in the body of the acrylic synthetic fibers. A most recommendable way for attaining this is such that a polymer comprising at least 70 wt. percent of polyacrylnitrile is wet spun into multifilaments which, in their wet gel state and subjected to a drying step, are brought into contact with said derivative by application thereof. By adopting this measure, considerably large quantity of said derivative can be applied to the fibers without any appreciable loss of the desirous textile characteristics such as favorable dyeing properties, dyeing fastness, strength, stretchability, hand feeling and the like.

In addition, the thus applied polyalkylene ether derivative is found to be highly durable to long extended boiling water treatment; dyeing treatment and repeated washings and laundering treatments. In these cases, a small part of the applied derivative or antistatic agent will be removed, but a substantial part thereof remains as a "residue."

The fibrous material thus fed with the derivative shows a remarkable and so-to-speak a permanent antistatic property.

According to our practical experiments, we have found that the initial dosing of said derivative to the polyacrylic fibers, on the one hand, and the residual quantity of the derivative within the fibers as measured upon boiling water treatment, on the other hand, can be expressed by way of example as shown in the attached drawing.

The initial dosing quantity mentioned throughout the present specification means such quantity of polyalkylene ether derivative which the fibers reserve therein upon the processing treatment according to the process of the invention, said quantity being measured relative to the dry weight of the material fibers.

The residual quantity in the above sense is that which is preserved upon a boiling water treatment extending for an hour. This quantity is also measured relative to the dry weight of the fibers. During said boiling treatment, a certain quantity of the derivative will be removed, but it has been found that still further appreciable removal will not generally be encountered, even when the fiber is subjected to further continued boiling treatment or to repeated washings and laundering treatments. As will be seen from the drawing, the residual quantity of the derivative will increase with an increase of the initial dosing. However, it should be noted that the residue rate (residual quantity/initial dosing) will decrease gradually. There will be a certain saturation value for a certain initial dosing. Beyond this value, an increase of the initial dosing will invite no appreciable increase in the residual quantity. This residual quantity may be called the "saturated pick-up" and the initial dosing corresponding to this pick-up will be defined as the "S-value" throughout the specification.

The S-value is an adsorption equilibrium quantity which has however a certain margin depending upon the kind and nature of the fiber material polymer, derivative, the solvent and the spinning conditions. As a general measure, the S-value for acrylic fibers generally amounts to 5-10%.

It has now amazingly been found that when the initial dose is smaller than the S-value, the desirous antistatic property will become very weak, while with the initial dose higher than the S-value, the antistatic performance of the treated fibers will be amazingly high. A preferred process according to the invention is based upon the above observation and is carried out advantageously so that the acrylic synthetic fibers of the above kind are treated with a polyalkylene ether derivative in such a way that the initial dose will amount to at least the saturated pick-up or adsorption value in the above sense. These saturated pick-up or adsorption values can be easily determined by simple preparatory experiments.

Upon treatment of the fibers in the wet gel state in the afore-mentioned manner, the fibers are dried, thereby fixing the polyalkylene ether derivative in position within the interior of the mass of each of the fibers to a sufficient degree of washfastness, and indeed, without any substantial loss of the originally owned favorable physical and chemical properties.

In the case of the liquid treatment, the selection of the initial dose of the antistatic agent or polyalkylene ether derivative is made in consideration of the bath concentration and the liquid pick-up quantity by the wet gel fibers. The residual quantity of the antistatic substance in the body of the fibers may be controlled substantially exclusively by adjusting the degree of mangling or centrifuging in the above-menitioned sense. As an example, when the mangling or centrifuging is adjusted to provide a 100% pick-up relative to the dry weight of the fibers upon immersion of the latter in its wet gel state in a treating bath, having a 15 wt. percent concentration to the derivative, the initial dose will amount to about 15%. With a reduced 75 pick-up of 50%, the initial dose will be about 7.5%.

When the principle of the invention is used in a continuous industrial process, the concentration of the treating bath must be higher than the initial dose, percent, relative to the wet gel filamentary fibers, preferably in the form of a tow, because the latter will introduce additional aqueous content to the bath composition. The fiber in its wet gel state will generally exhibit a 40 wt. percent, or higher, aqueous content, for instance, as measured directly after the spinning step of the fiber.

The conventionally employed stretching process may be carried out either in advance or after the contacting treatment of the fibers with the polyalkylene ether derivative. The acrylic fiber tow may be subjected to a heat treatment, and cut to proper lengths, such as, for example, 60-100 mm., the thus cut fibers being opened, as is conventional, to fiber webs.

It has been found that the polyalkylene ether derivatives thus incorporated in polyacrylic fibers are substantially durable to hot water treatment after finishing repeatedly applied washings and laundering treatments. Therefore, the amount of the incorporated polyalkylene ether derivative can be preserved in a quantity substantially equal to the initial dose in the treated filamentary fibers even upon frequently repeated laundering treatments. Thus, it may definitely be said that the antistatic performance of the acrylic fibers is improved in accordance with the novel teaching proposed by the present invention and is, so-to-speak, semi-permanent.

The following, several preferred numerical examples will be given for a better understanding of the invention, wherein the antistatic performance of the fibers is given in each case in ohms by measurement of the characteristic surface resistance referred to briefly as "resistance" hereinafter, of a web composed of these fibers. The measurement was performed substantially as prescribed in the U.S. Standards, AATCC 76-1964. The measuring instrument used for this purpose was a "TR-65 Electrometer" manufactured by Takeda Riken Kabushiki Kaisha, Tokyo. The measuring sample composed of well opened fibers, 2 gr. The fiber cut length amounted to 6 cm. The sample container was a round cylindrical case of 50 cm., I.D., and having a 40 mm. height. A stationary cylindrical electrode was used, its O.D. being 40 mm.; and its thickness being 0.5 mm. The opposite movable electrode had an O.D. of 40 mm. and a height of 30 mm. The resistance value was measured on an ohmmeter inserted in a measuring circuit including said two electrodes.

The relative humidity prevailing in the measuring chamber was maintained at 65%.

The judgement between the effectiveness and ineffectiveness of the desired antistatic performance was made in the following way: various fibrous webs of different resistance were shaped into respective threads from which knits were manufactured and tested upon wearing personally for the determination of the critical resistance value below which the unfavorable electrical discharge noises were not sensed by human ears. This critical value was found to be  $10^{11}$  ohms. Then, the sample webs were boilingly dyed and then subjected to 10 times repeated washing treatments upon which the resistance value was measured in the aforementioned way. In the following examples, the acceptable upper limit of resistance value was set to the above-specified value of  $10^{11}$  ohms. The dyeing was carried out with a conventional cationic dyestuff in the form of an aqueous solution as its boiling temperature for an hour. For the washing treatments, a 0.3%-aqueous solution of sodium alkylbenzenesulfonate was used at 40° C. for 30 minutes, the bath ratio being 1:50, while using a "Launder-O-Meter." The dyed textile was then washed in a cold water bath for 5 minutes and then dried. It was assumed that this treatment corresponds to five regular washings.

#### EXAMPLE 1

An acrylonitrile copolymer comprising acrylonitrile 92.0 wt. percent, vinyl acetate 5.0 wt. percent and acryl-

amide 3.0 wt. percent, dissolved in dimethylformamide, was mixed with a compound corresponding to dodecyl phenol occupying 2.5 wt. percent of the polymer and with 180 mols of ethylene oxide, and the resulting mixture was intimately mixed together and dry spun into multifilaments from which a web was manufactured. Resistance of the web as formed, amounted to  $7 \times 10^{10}$  ohms. After dyeing and 10 repeated washings, the web showed a resistance of  $5 \times 10^{11}$  ohms.

As a comparative test, the resistance of a multifilament web admixed with none of the polyoxyalkylene ether derivative was measured under similar conditions and amounted to  $4 \times 10^{14}$  ohms.

#### EXAMPLE 2

An acrylonitrile copolymer comprising acrylonitrile 91.7 wt. percent, methyl acrylate 3.0 wt. percent, acrylamide 5.0 wt. percent and sodium metallylsulfonate 0.3 wt. percent and dissolved in sodium rhodanate was mixed with a compound corresponding to octyl phenol which corresponds in turn to 6 wt. percent of the polymer and 2 mols of ethylene oxide, and mixed together intimately and then wet spun into multifilaments. A web manufactured therefrom showed in its resistance  $2 \times 10^{11}$  ohms as spun. Upon being dyed and washed ten times, the web showed a resistance of  $8 \times 10^{11}$  ohms.

As a comparative test, a similar web was prepared without addition of the polyoxyalkylene ether derivative thereto and showed a resistance of  $8 \times 10^{14}$  ohms.

#### EXAMPLE 3

A solution of the acrylonitrile copolymer of Example 1 dissolved in nitric acid, was mixed with a compound comprising dodecyl alcohol corresponding to 4 wt. percent of the polymer and added with 10 mols of ethylene oxide. The resulting mixture was mixed together evenly and wet spun to multifilaments. A web prepared therefrom showed a resistance of  $2 \times 10^9$  ohms, and upon being dyed and washed 10 times  $4 \times 10^{10}$  ohms.

As a reference, a similar web was prepared with no polyoxyalkylene ether derivative and the measured resistance was  $6 \times 10^{14}$  ohms.

#### EXAMPLE 4

A solution of the same acrylonitrile copolymer disclosed in Example 2 in sodium rhodanate was mixed with a compound comprising polypropylene glycol corresponding to 7 wt. percent of the polymer and having an average degree of polymerization of 15 and 18 mols of ethylene oxide. The thus resulting mixture was mixed together thoroughly and wet spun to multifilaments. A web prepared therefrom showed a resistance as spun of  $1 \times 10^{10}$  ohms and upon being dyed and washed 10 times  $9 \times 10^{10}$  ohms.

As a comparative test, a similar web was prepared, without addition of polyoxyalkylene ether derivative thereto, whose resistance was  $6 \times 10^{14}$  ohms.

#### EXAMPLE 5

A solution of an acrylonitrile copolymer comprising acrylonitrile 89.5 wt. percent, methyl acrylate 5.0 wt. percent, methyl methacrylate 5.0 wt. percent and sodium parastyrenesulfonate 0.5 wt. percent dissolved in nitric acid was wet spun into multifilaments which were then washed and subjected to an 8-times elongation, so as to provide a multifilament tow in the wet gel state.

The tow was immersed in an aqueous solution of polyalkylene ether derivative for 30 minutes, the initial dosing being shown in Table I, squeezed, dried and then steamed at 120° C. The filament had a mean denier of 3. The resistance and other properties of the web are shown in Table I.

TABLE I

| Sample designation of polyalkylene ether | Initial dosing rate, percent | Rate of pick-up, percent | Treated web     | Resistance value, ohms                     |                         |                                |
|------------------------------------------|------------------------------|--------------------------|-----------------|--------------------------------------------|-------------------------|--------------------------------|
|                                          |                              |                          |                 | Upon dyeing and 25 times repeated washings | Tensile strength, g./d. | Elongation percentage, percent |
| Blank                                    |                              |                          |                 | $7 \times 10^4$                            | $3 \times 10^4$         | 28.2                           |
| "A"                                      | 4.8                          | 3.7                      | $5 \times 10^4$ | $2 \times 10^4$                            | 3.6                     | 29.4                           |
|                                          | 10.1                         | 6.4                      | $1 \times 10^9$ | $5 \times 10^4$                            | 3.3                     | 31.5                           |
|                                          | 14.6                         | 8.1                      | $3 \times 10^8$ | $9 \times 10^4$                            | 3.2                     | 33.2                           |
|                                          | 24.7                         | 8.6                      | $9 \times 10^8$ | $8 \times 10^4$                            | 2.8                     | 36.1                           |
| "B"                                      | 3.6                          | 2.8                      | $2 \times 10^9$ | $7 \times 10^4$                            | 3.5                     | 29.6                           |
|                                          | 9.8                          | 6.2                      | $7 \times 10^9$ | $2 \times 10^4$                            | 3.2                     | 30.6                           |
|                                          | 15.0                         | 8.0                      | $6 \times 10^9$ | $7 \times 10^4$                            | 3.1                     | 32.3                           |
|                                          | 25.7                         | 8.2                      | $8 \times 10^9$ | $6 \times 10^4$                            | 2.7                     | 34.7                           |
| "C"                                      | 4.2                          | 3.5                      | $7 \times 10^4$ | $3 \times 10^4$                            | 3.6                     | 29.1                           |
|                                          | 10.5                         | 6.4                      | $5 \times 10^4$ | $9 \times 10^4$                            | 3.4                     | 31.7                           |
|                                          | 14.5                         | 7.9                      | $2 \times 10^9$ | $6 \times 10^4$                            | 3.3                     | 32.0                           |
|                                          | 26.4                         | 8.1                      | $4 \times 10^8$ | $1 \times 10^4$                            | 2.9                     | 35.2                           |

In the foregoing Table I, the derivatives "A"- "C" represent the following compounds:

- "A" ----- Dodecyl alcohol added with 20 mols of ethylene oxide.  
 "B" ----- Methylene-bis-phenol added with 5 mols of propyleneoxide.  
 "C" ----- Castor oil added with 10 mols of ethylene oxide.

The dyeing was carried out using the cationic dyestuff "Astrazon Red RL" (manufactured and sold by Farbenfabriken Bayer A.G., Leverkusen, Germany) in a quantity of 1% of the total weight of the fibers under boiling conditions for an hour, with a bath ratio 1:40. Saturated absorption: about 8%. Initial supply quantity therefor (S-value): about 14%.

In the case of the antistatic agent "A" with its initial supply quantity 10.1% and in spite of the existence of 6.4% of the antistatic agent within the fibers, the resistance values as measured upon spinning and upon washing treatments were substantially similar to those of the blank products, since the taken-up quantity was less than the said saturated value. On the contrary, with the initial dosing of 14.6%, the resistance as measured upon dyeing and repeated washes was rather low, representing a permanent antistatic performance.

As for the remaining agents "B" and "C," similar observations could be made.

#### EXAMPLE 6

Similar tows were prepared as in the foregoing Example 5. The remaining treatments were also similar to those mentioned therein. The initial dosing amounted to about 15% of the saturation value.

TABLE II

| Sample designation of polyalkylene ether | Initial supply quantity, percent | Incorporated quantity, percent | Resistance value, ohms |                                            |
|------------------------------------------|----------------------------------|--------------------------------|------------------------|--------------------------------------------|
|                                          |                                  |                                | Treated web            | Upon dyeing and 25 times repeated washings |
| Blank                                    |                                  |                                |                        | $2 \times 10^4$                            |
| "D"                                      | 14.8                             | 7.9                            | $6 \times 10^9$        | $5 \times 10^4$                            |
| "E"                                      | 15.3                             | 8.4                            | $1 \times 10^9$        | $3 \times 10^4$                            |
| "F"                                      | 15.5                             | 9.1                            | $7 \times 10^8$        | $4 \times 10^4$                            |
| "G"                                      | 14.5                             | 8.3                            | $3 \times 10^9$        | $8 \times 10^4$                            |

In these tests, the derivatives "D"- "G" were as follows:

- 35 "D" ----- Octylalcohol added with 2 mols of ethylene oxide.  
 "E" ----- Dodecyl phenol added with 180 mols of ethylene oxide.  
 40 "F" ----- Stearic acid added with 20 mols of ethylene oxide.  
 "G" ----- Sorbitan oleate added with 13 mols of ethylene oxide.

#### EXAMPLE 7

45 A solution of acrylonitrile copolymer comprising acrylonitrile 92.0 wt. percent, vinyl acetate 5.0 wt. percent and acrylamide 3.0 wt. percent and dissolved in sodium rhodanate was wet spun, washed and subjected to about 700% elongation, so as to provide tows in a wet gel state.

50 These tows were immersed in an aqueous solution of polyalkylene ether derivative "A" for 30 minutes, squeezed, dried and steamed at 120° C. The fibers thus obtained had a mean denier of 15. The webs prepared therefrom showed the following characteristics as shown in Table III.

TABLE III

| Sample designation of polyalkylene ether | Initial supply quantity, percent | Incorporated quantity, percent | Resistance value, ohms |                                            |                         |                       |
|------------------------------------------|----------------------------------|--------------------------------|------------------------|--------------------------------------------|-------------------------|-----------------------|
|                                          |                                  |                                | Treated web            | Upon dyeing and 25 times repeated washings | Tensile strength, g./d. | Elongation percentage |
| Blank                                    |                                  |                                | $8 \times 10^4$        | $2 \times 10^4$                            | 2.9                     | 30.5                  |
| "A"                                      | 4.7                              | 3.8                            | $1 \times 10^9$        | $9 \times 10^4$                            | 3.1                     | 29.2                  |
|                                          | 7.5                              | 4.9                            | $5 \times 10^9$        | $8 \times 10^4$                            | 2.5                     | 31.5                  |
|                                          | 11.0                             | 6.2                            | $3 \times 10^9$        | $4 \times 10^4$                            | 2.4                     | 33.0                  |
|                                          | 20.7                             | 6.4                            | $4 \times 10^8$        | $6 \times 10^4$                            | 2.0                     | 33.8                  |

Test results are shown in Table II. Resistances were less than  $10^{11}$  ohms, which means a sufficient permanent antistatic performance.

75 In these samples, the saturating or saturated absorption amounted to about 6% and the initial dosing necessary therefor was about 11%.

With an initial dosing of 7.5%, the resistance values were substantially similar to those of the blank products since the dose was substantially smaller than the saturating threshold. With an initial dose of 11.0%, however, the treated fibrous products showed a sufficient antistatic performance.

## EXAMPLE 8

A solution of an acrylonitrile copolymer comprising 91.7 wt. percent acrylonitrile, methyl acrylate 3.0 wt. percent, acrylamide 5.0 wt. percent and sodium metallyl sulfonate 0.3 wt. percent, dissolved in nitric acid, was wet spun and then washed and subjected to a 700% elongation, so as to provide multifilaments in the wet gel-like state.

These filaments were dipped for 30 minutes in an aqueous solution containing compound "H" which comprises phenol added with 10 mols of propylene oxide and 15 mols of ethylene oxide, squeezed and dried. The multifilaments, 2 denier per filament, in the form of a bundle, 75 denier, were processed to a plain weave fabric and the resulting resistance values were measured. The results are shown in Table IV.

TABLE IV

| Sample designation of polyalkylene ether | Initial supply quantity, percent | Incorporated quantity, percent | Treated web        | Resistance value, ohms                     |                                          | Elongation percentage of filament yarn |
|------------------------------------------|----------------------------------|--------------------------------|--------------------|--------------------------------------------|------------------------------------------|----------------------------------------|
|                                          |                                  |                                |                    | Upon dyeing and 25 times repeated washings | Tensile strength of filament yarn, g./d. |                                        |
| Blank                                    |                                  |                                |                    | 6×10 <sup>14</sup>                         | 3×10 <sup>14</sup>                       | 3.4                                    |
| "H"                                      | 3.1                              | 2.5                            | 2×10 <sup>10</sup> | 4×10 <sup>14</sup>                         | 3.6                                      | 21.3                                   |
|                                          | 5.9                              | 4.1                            | 7×10 <sup>9</sup>  | 1×10 <sup>14</sup>                         | 3.3                                      | 22.5                                   |
|                                          | 9.2                              | 5.5                            | 1×10 <sup>9</sup>  | 8×10 <sup>10</sup>                         | 3.0                                      | 21.6                                   |
|                                          | 15.3                             | 5.7                            | 5×10 <sup>10</sup> | 1×10 <sup>11</sup>                         | 2.8                                      | 25.4                                   |

The embodiments of the invention in which an exclusive property or privilege is claimed are as follows:

1. A process for treating acrylic synthetic fibers to impart permanent antistatic properties thereto, said acrylic synthetic fibers being composed of a polymer selected from the group consisting of a homopolymer of acrylonitrile and copolymers of acrylonitrile with at least one unsaturated monomer copolymerizable therewith, said copolymer containing at least 70% by weight acrylonitrile, said process comprising contacting said fibers which are in a gel state, prior to drying, with a first amount of at least one polyalkylene derivative represented by the formula:



wherein R is a hydrophobic organic radical having from 6 to 40 carbon atoms derived from a compound containing a —OH or a —COOH group, by removing said —OH or said —COOH, said compound being selected from the group consisting of octyl alcohol, dodecyl alcohol, hexadecyl alcohol, octadecyl alcohol, octadecenyl alcohol, octylphenol, dodecylphenol, stearic acid monoglyceride, ricinoleic acid triglyceride, sorbitan oleate, sorbitan distearate, octanoic acid, dodecanoic acid,  $\alpha$ -hydroxy decanoic acid, sebacic acid,  $\alpha$ - or  $\omega$ -dihydroxy octane and methylene bisphenol; R' is hydrogen or methyl; X is O or COO; n is an integer of 2-200 and m is an integer of from 1 to 6; said first amount being determined by measuring, under the conditions of said contacting step, the maximum amount of said derivative which said fibers will adsorb and retain when the fibers are boiled in water for 1 hour, and then measuring the second amount of said derivative which must be contacted with said fibers to provide said maximum amount, wherein said first amount is greater than said second amount.

2. The process of claim 1 wherein said maximum amount varies from 5 to 10% by weight of said derivative, based on the dry weight of said fibers.

3. The process of claim 1 wherein said copolymer

55  
60  
65  
70

50  
45  
40  
35

erizable monomer is selected from the group consisting of methacrylic acid, butyl vinyl ether, acrylic acid ester, methacrylic acid ether, vinyl ether, vinyl acetate ester, styrene sulfonic acid, sodium styrene sulfonate, sodium allylsulfonate and sodium methallyl sulfonate.

5. The process of claim 1 wherein said hydrophobic organic radical is derived from castor oil, tallow or a fatty acid.

6. The process of claim 1 wherein said fibers are immersed in an aqueous solution of said derivative at a temperature of from 20 to 30° C. and then centrifuged at room temperature.

7. The process of claim 1 wherein said fibers are directly contacted with said derivative in liquid form.

8. The process of claim 1 wherein said fibers in a gel state comprise fibers having at least a 40 wt. percent aqueous content.

9. In a process for producing acrylic synthetic fibers including the steps of:

(1) forming continuous filaments by wet-spinning an acrylonitrile polymer selected from the group con-

sisting of a homopolymer of acrylonitrile and copolymers of acrylonitrile with at least one unsaturated monomer copolymerizable therewith, said copolymer containing at least 70% by weight of acrylonitrile; (2) washing said continuous filaments; and (3) drying the washed continuous filaments to produce said acrylic synthetic fibers;

40  
45  
40  
35

the improvement comprising producing synthetic acrylic fibers having permanent antistatic properties by contacting said continuous filaments, prior to said drying step (3), which continuous filaments are in a wet gel state, with an aqueous solution containing a first amount of at least one polyalkylene ether derivative represented by the formula:



wherein R is a hydrophobic organic radical having from 6 to 40 carbon atoms derived from a compound containing —OH or a —COOH group by removing said —OH or said —COOH group, said compound being selected from the group consisting of octyl alcohol, dodecyl alcohol, hexadecyl alcohol, octylphenol, dodecylphenol, stearic acid monoglyceride, ricinoleic acid triglyceride, sorbitan oleate, sorbitan distearate, octanoic acid, dodecanoic acid,  $\alpha$ -hydroxy decanoic acid, sebacic acid, or  $\omega$ -dihydroxy octane and methylene bisphenol; R' is hydrogen or methyl; X is O or COO; n is an integer of 2-200 and m is an integer of from 1 to 6; said first amount being determined by measuring, under the conditions of said contacting step, the maximum amount of said derivative which said fibers will adsorb and retain when the fibers are boiled in water for one hour, and then measuring the second amount of said derivative which must be contacted with said fibers to provide said maximum amount, wherein said first amount is greater than said second amount.

10  
15  
20  
25  
30  
35  
40  
45  
50  
55  
60  
65  
70  
75

**11**

said maximum amount, wherein said first amount is greater than said second amount.

**10.** The process of claim **9** wherein said maximum amount varies from 5 to 10% by weight of said derivative, based on the dry weight of said fibers.

**11.** The process of claim **10** wherein said continuous filaments are subjected to a stretching step after said washing step and then subjected to said contacting step and then dried.

**12.** The process of claim **11** wherein said hydrophobic organic radical is derived from castor oil, tallow or a fatty acid.

**13.** The process of claim **11** wherein said washing step comprises washing said continuous filaments with water and wherein the temperature of said contacting step is from 20 to 30° C. and wherein after said contacting step, the resulting continuous filaments are centrifuged at room temperature.

**12****References Cited****UNITED STATES PATENTS**

|             |         |          |          |
|-------------|---------|----------|----------|
| 2,829,066   | 4/1958  | Murdock  | 117—7    |
| 2,920,980   | 1/1960  | Mooberry | 117—65   |
| 5 2,965,678 | 12/1960 | Sundberg | 260—615  |
| 3,329,644   | 7/1967  | Baur     | 260—32.6 |

**FOREIGN PATENTS**

|            |        |         |             |
|------------|--------|---------|-------------|
| 10 616,953 | 4/1962 | Belgium | 260—Dig. 17 |
|------------|--------|---------|-------------|

**OTHER REFERENCES**

Haye K. M.: American Dyestuff Reporter (June 7, 1954), pp. 368—371.

15 JOSEPH L. SCHOFER, Primary Examiner

C. A. HENDERSON, JR., Assistant Examiner

**U.S. CL. X.R.**

260—85.5 S, 88.7 B, Dig. 15, 17, 21; 264—178 F, 182